

**United States Patent [19]****Naito****Patent Number: 4,710,450****Date of Patent: Dec. 1, 1987**

[54] **PHOTOGRAPHIC ELEMENT COMPRISING AT LEAST TWO EXOTHERMIC ELECTROCONDUCTIVE LAYERS**

[75] Inventor: **Hideki Naito, Minami-ashigara, Japan**

[73] Assignee: **Fuji Photo Film Co., Ltd., Kanagawa, Japan**

[21] Appl. No.: **829,033**

[22] Filed: **Feb. 13, 1986**

[30] **Foreign Application Priority Data**

Feb. 13, 1985 [JP] Japan ..... 60-26055

[51] **Int. Cl. 4** ..... **G03G 15/12**

[52] **U.S. Cl.** ..... **430/351; 430/353;**  
..... **430/62**

[58] **Field of Search** ..... **430/110, 56, 945, 60,**  
..... **430/62**

[56] **References Cited**

**U.S. PATENT DOCUMENTS**

4,460,636 7/1984 Watanabe ..... 430/945  
4,525,722 6/1985 Sachdev et al. ..... 430/945  
4,578,322 3/1986 Sawamura et al. ..... 430/945

*Primary Examiner*—John L. Goodrow  
*Attorney, Agent, or Firm*—Sughrue, Mion, Zinn,  
Macpeak, and Seas

[57] **ABSTRACT**

A photographic element comprising photosensitive and image-receiving layers on a support further includes a primary exothermic electroconductive layer serving as a heating element and an auxiliary exothermic electroconductive layer thereon, wherein the primary conductive layer containing conductive substance like carbon black so that it is heated upon electric conduction, contributing to heat development.

**17 Claims, No Drawings**

**PHOTOGRAPHIC ELEMENT COMPRISING AT LEAST TWO EXOTHERMIC ELECTROCONDUCTIVE LAYERS**

**BACKGROUND OF THE INVENTION**

This invention relates to a photographic element for use in a process for forming an image through heat development, and more particularly, to such a photographic element having an exothermic layer.

Heat developable photosensitive materials and heat development process are well known in the art and described in the literature, inter alia, "Fundamentals of Photographic Engineering", Corona Publishing K.K., Tokyo, Japan (1979), pages 553-555; "Image Information", April 1978, page 40; Neblette's Handbook of Photography and Reprography, 7th ed., Van Nostrand Reinhold Company, pages 32-33; U.S. Pat. Nos. 3,152,904, 3,301,678, 3,392,020, and 3,457,075; British Pat. Nos. 1,131,108 and 1,167,777; and Research Disclosure, June 1978, pages 9-15 (RD-17029).

A process for transferring a mobile dye imagewise formed by heat development to an image-receiving layer by heating and image-receiving materials used therefor are described in Japanese Patent Application Kokai Nos. 58-58543, 58-79247, and 59-168439, inter alia.

Heating of these heat-developable photosensitive materials and image-receiving materials (both generally referred to as photographic materials, hereinafter) may be carried out by a number of methods including contacting of photographic materials with a heat block having a great capacity; direct heating of photographic materials by laser and infrared irradiation, ultrasonic heating, high frequency heating or the like; and passing of photographic materials through heated gas. These methods are, however, not successful in achieving satisfactory results because of their shortcomings. For instance, in the use of a heat block, is time and power consuming to accomplish a uniform temperature distribution throughout the heat block, and insufficient contact prevents smooth uniform heat transfer to the photographic material. The use of radiation such as by a laser beam is disadvantageous in that a large sized apparatus is required or a compact system is difficult to incorporate. The use of heated gas is time consuming because the gas has essentially a low heat capacity.

To overcome these shortcomings, the use of an exothermic electroconductive layer in combination with a heat developable photosensitive layer was proposed as disclosed in, for example, U.S. Pat. No. 206,368 and Japanese Patent Kokai No. 48-66442.

Also, a variety of positive electroconductive layers (which herein designate electroconductive layers whose electric resistance increases with a temperature rise) intended for plane heaters were developed as disclosed in, for example, Japanese Patent Application Kokai Nos. 49-82734, 49-82735, 51-13991, 51-39742, 51-39743, and 52-87694.

These methods aim to prevent overheating by taking advantage of the nature of these materials, i.e., their electric resistance increases with a temperature rise, and employ these materials as plane heaters and in snow melting systems. It is possible to apply these positive electroconductive layer to photographic materials and such an application is described, for example, in Japanese Patent Application No. 58-229377.

Any desired choice of design may be made on an exothermic electroconductive layer so as to meet the intended application whether it is of the positive type as mentioned above, of the negative type wherein the electric resistance of an electroconductive layer decreases with a temperature rise, or of the neutral type wherein resistance does not depend on temperature. With respect to a binder used in such a layer, a choice may be made between hydrophilic binders and hydrophobic polymeric binders combined with organic solvents, depending on the desired properties of the electroconductive layer.

When these exothermic electroconductive layers are used in combination with heat-developable photosensitive layers as photographic materials, the electroconductive layers must be imparted with properties other than electroconductive properties. In the case of a sheet- or roll-shaped sample, interfacial adhesion must be prevented between a photosensitive layer and an electroconductive layer when these layers overlap one another, marring on the electroconductive layer surface must be prevented during mechanical transfer of the sample, and an improvement is required in overcoming variation of resistance value when the sample and developing equipment are held under different ambient conditions including relative humidity and temperature.

Such considerations are essential to accomplish stable heat development and transfer of a mobile dye by heating and not fully met by the conventional photographic material. There is the continuing need for a further improvement in this respect.

**SUMMARY OF THE INVENTION**

It is, therefore, an object of the present invention to provide a novel and improved photographic element capable of stable uniform heat development or transfer of a mobile dye by heating wherein when sheets of heat-developable photographic material having electroconductive and photographic layers are placed one on another for shelf storage, adhesion between adjoining electroconductive and photographic layers or between adjoining electroconductive layers is prevented as well as marring and crazing owing to physical contact, pressure or other factors, and the dependency of electric resistance on humidity is avoided.

According to the present invention, there is provided a photographic element comprising at least two exothermic electroconductive layers and a photosensitive layer and/or an image-receiving layer on a support.

**DETAILED DESCRIPTION OF THE INVENTION**

The photographic element according to the present invention includes at least two exothermic conductive layers. The term conductive as used throughout the disclosure means that the layers are electroconductive.

Among the at least two exothermic conductive layers, at least one layer is an exothermic conductive layer having the function of a heating element (to be also referred to as a primary conductive layer, hereinafter). In addition to the primary conductive layer, there is provided at least one auxiliary exothermic conductive layer having a desired combination of physical properties for the intended application (to be also referred to as an auxiliary layer, hereinafter). The auxiliary layer is provided on the primary conductive layer, preferably in direct contact therewith.

The materials from which the exothermic conductive layers according to the present invention are formed may be any of the materials described in the preamble.

With respect to electric resistance, the primary conductive layer having the function of a heating element should have a volume resistance of  $10^{-4}$  to 10 ohm-cm and the auxiliary layer provided should additionally have a volume resistance of  $10^{-1}$  to  $10^4$  ohm-cm.

The auxiliary layer is rendered conductive in the present invention because it is readily made in contact with an electrode to ensure electric conduction. Otherwise, an additional lead must be attached to the primary conductive layer, resulting in a complicated structure, difficulty in manufacture, and less reliable electric conduction.

The primary conductive layer having a volume resistance of  $10^{-4}$  to 10 ohm-cm may be prepared by any of the well-known techniques.

The conductive layers may be of any desired construction, and preferably contain a conductivity-imparting substance in the form of fine particles dispersed in a binder.

Typical examples of the conductivity-imparting substances include metals such as iron, copper, silver, nickel, platinum, etc., alloys such as those alloys based on nickel and/or chromium also known as Nichrome and Kanthal; noble metal alloys such as platinum-rhodium alloys, silicon carbide, molybdenum silicide, and oxide semiconductors such as zirconia ( $ZrO_2$ ), zinc oxide, titanium dioxide, and thorium ( $ThO_2$ ), graphite and carbon black. Most preferred among these are graphite and carbon black because of their low cost. Conductive carbon black is known among the carbon black species while any types of carbon black may be equally employed. These types of carbon black are described in Carbon Black Annual and J. B. Donnet & A. Voet, "Carbon Black", Marcel Dekker (1976), and commercially available from Columbian Carbon Company, Mitsubishi Chemical Industry K.K., and other manufacturers.

Preferred among these types of carbon black are those having a dibutyl phthalate (DBP) oil absorption of more than 80 cc/100 grams as measured by Procedure A or B prescribed in JIS K 6221. These preferred carbon blacks are readily chosen and available from the carbon catalogs of Cabot Corporation, Lion Akzo K.K., Colombian Carbon Japan K.K., and other manufacturers. Some illustrative, but non-limiting examples are BLACK PEARLS 1300, BLACK PEARLS 1000, BLACK PEARLS 880, BLACK PEARLS 700, BLACK PEARLS 2000, VULCAN XC-72, VULCAN P, VULCAN 9, REGAL 300R, ELFTEX PELLETS 115, ELFTEX 8, ELFTEX 12, STERLING SO, and STERLING V all available from Cabot Corporation; KETJEN BLACK EC manufactured by Japan EC K.K. (marketed from Lion Akzo K.K.); ROYAL SPECTRA, NEO SPECTRA MARK I and II, NEO SPECTRA AG, SUPERBA (NEO MKII), NEO SPECTRA MARK IV, RAVEN 5000, RAVEN 7000, RAVEN 5750, RAVEN 5250, RAVEN 3500, RAVEN 3200, RAVEN 1040, RAVEN 890 POWDER, RAVEN 890H POWDER, RAVEN 825 BEADS, RAVEN 500, CONDUCTEX 40220, CONDUCTEX 975 BEADS, CONDUCTEX 900 BEADS, CONDUCTEX SC, RAVEN H20 POWDER, RAVEN C BEADS, RAVEN 22 POWDER, RAVEN 16 POWDER, and RAVEN 14 POWDER all available from Columbian Carbon Japan K.K.

Conductive layers containing such carbon black having a high DBP oil absorption vary little their resistance with a change of ambient humidity. The greater DBP oil absorption, more outstanding is the effect. In the preferred embodiment of the present invention, carbon blacks are used having a DBP oil absorption of more than 100 cc/100 grams, most preferably more than 150 cc/100 grams.

The binders used in the primary conductive layer in the practice of the present invention are preferably hydrophilic. The hydrophilic binders are typically transparent and translucent hydrophilic colloids, for example, natural substances, for example, proteins such as gelatin, gelatin derivatives, cellulose derivatives, etc. and polysaccharides such as starch and gum arabic, and synthetic polymers, for example, water-soluble polyvinyl compounds such as polyvinyl alcohol and polyvinyl pyrrolidone and acrylamide polymers. Particularly useful among them are gelatin and polyvinyl alcohol, with gelatin being most preferred.

The conductive layers may be applied by coating with the sole use of a hydrophilic conductive high-molecular weight compound which has both the functions of a conductivity imparting substance and a hydrophilic binder. Exemplary of the conductive high-molecular weight compounds there may be given cationic high-molecular weight electrolytes such as polypiperidinium chloride, polyvinylbenzyl trimethylammonium chloride, etc.

It is also possible to use conductive fine particles in admixture with conductive high-molecular weight compounds.

The conductive films formed from the conductive fine particles and the conductive high-molecular weight compounds individually or in admixture of any two or more of them have an electric resistance which may be controlled to any desired value by a suitable choice of the ratio of conductive material to binder, dispersion method, the particular type of binder used or the like. Such control is well known in the art and described in the afore-mentioned literature and technical documents of carbon black manufacturers.

The amount of the conductive component used in the conductive films generally ranges from 10 to 90% by weight, preferably from 15 to 85% by weight. Better results are obtained particularly when carbon black is used in an amount of about 0.1 to about 50 grams/m<sup>2</sup>, preferably about 0.5 to about 20 grams/m<sup>2</sup> as the conductive fine particles. In this case, the content of carbon black in the conductive film ranges from about 10 to about 90% by weight, preferably from about 15 to about 80% by weight.

At least one auxiliary layer formed in addition to the primary conductive layer may have any desired organization depending on the particular purposes.

Preferred examples of the auxiliary layer are given below. However, it should be noted that the present invention is not limited to the following examples as long as at least two conductive layers are provided.

A. For the purpose of preventing adhesion between conductive and photographic layers or between conductive layers held in mutual contact during shelf storage.

Generally, a binder different from that used in the photographic layer is desirably used although some changes occur depending on the components of which the photographic layer or primary conductive layer is formed. For example, when the binder used in the photo-

photographic layer is gelatin, hydrophilic polymeric binders of different type are partially or solely used, such as polyvinyl alcohol, polyvinyl pyrrolidone, albumin, and gum arabic.

Also usable are hydrophobic high-molecular weight compounds. Hydrophobic high-molecular weight compounds in latex form may also be used in admixture with hydrophilic polymers. Furthermore, water- or oil-repellent surface-active agents may be used.

Independent of the particular type of polymer used, particles having a size of the order of several micra are also useful as a so-called matte agent. Examples of the matte agents include latices of synthetic high-molecular weight compounds, finely divided inorganic materials such as silica, and coarse particulates of metals, graphite and carbon black.

The auxiliary layers formed in this manner preferably have a thickness of about 0.1 to 20  $\mu\text{m}$ , more preferably about 0.3 to 5  $\mu\text{m}$ , and an electric resistance of about  $10^{-1}$  to  $10^4$  ohm-cm. To set the electric resistance within this range, any of the afore-mentioned materials may be used as the conductivity-imparting substance. The desired resistance may be obtained by suitably choosing the type and amount of such conductive substance.

When the auxiliary layer is provided for the captioned purpose, it may have an electric resistance substantially equal to or higher than that of the primary conductive layer.

B. For the purpose of protecting the surface of the primary conductive layer to prevent marring and crazing due to physical contact, pressure or the like.

The presence of mars and other defects on the primary conductive layer causes non-uniform exothermal distribution, rendering uniform development difficult to achieve. The auxiliary layer provided for the captioned purpose need not contribute to exotherming or heating by electric conduction and desirably has a higher resistance, most preferably at least one and one-half folds higher resistance than the primary conductive layer. Any desired electric resistance may be given in the same manner as described in (A). The auxiliary layer may be formed of any desired binders and have any desired thickness depending on the depth of likely defects, but generally a thickness in the range from about 0.1 to 20  $\mu\text{m}$ .

For the purpose of preventing crazing under pressure or stress, plastic binders are preferably used and, for example, those polymeric binders having a relatively low glass transition temperature  $T_g$  are useful. Polymeric binders having a relatively high  $T_g$  are also useful insofar as they are combined with plasticizers to form a plasticized film. For example, when gelatin is used as the binder for the auxiliary layer, it may be combined with plasticizers, for example, hydrophilic compounds such as water, urea derivatives, sulfonamide derivatives, etc., high molecular weight compounds having low  $T_g$  such as butadiene-styrene rubber (SBR) latex, dispersions in high-boiling solvents of compounds known as polymer plasticizers such as dibutyl phthalate (DBP) and tricresyl phosphate (TCP).

C. For the purpose of forming a humidity-resistant exothermic conductive layer by providing a humidity-resistant auxiliary layer on the surface of the primary conductive layer.

Since the auxiliary layer itself need not contribute to exotherming upon electric conduction, it may have an electric resistance equal to or higher than that of the

primary conductive layer. Any desired electric resistance may be given in the same manner as described in (A).

The binders from which the auxiliary layer is formed are preferably hydrophobic synthetic high-molecular weight compounds, for example, such polymers as polyesters, polycarbonates, poly(cellulose acetate), polyethylene butyral and formal derivatives, and polyamide derivatives.

The photographic element of the present invention is applicable to not only heat-developable photosensitive materials comprising a photosensitive silver halide, binder, organic silver salt oxidizing agent, and reducing agent on a support for producing black and white images, but also heat-developable photosensitive materials comprising a photosensitive silver halide, binder, and a dye-providing substance capable of producing or releasing a mobile dye in direct or counter proportion to the reduction of the photosensitive silver halide to silver at elevated temperatures on a support for producing color images, as well as image-receiving materials or dye-fixing materials for receiving the mobile dye produced or released from these color image-producing heat-developable photosensitive materials under heat through transfer mechanism.

In the practice of the present invention, the conductive layer (including both the primary conductive layer and auxiliary layer) and the photographic layer including photosensitive and image-receiving layers may be provided on the same or opposite sides of a support. Alternatively, they may be provided on separate supports wherein the conductive layer on one support may be placed on the photosensitive or image-receiving material on the other support into an integral assembly at any appropriate point of time. That is, any form may be taken insofar as heat produced by electric conduction is transferred to the photographic layer to heat it to a temperature necessary for development or image transfer. It is preferred to apply the conductive and photographic layers on opposite sides of a common support because the resulting photographic material is given a better curling balance. This arrangement is particularly preferable when the binder used in the conductive layer is water soluble because the resulting photographic material has layers of the same type formed on opposite sides of a support.

Some illustrative, but non-limiting arrangements of the conductive layers and the photosensitive or image-receiving layers are:

conductive layer/support/photosensitive or image-receiving layer,  
support/photosensitive or image-receiving layer/conductive layer, and  
support/photosensitive or image-receiving layer/intermediate layer/conductive layer.

The silver halides used in the present invention include silver chloride, silver bromide, silver iodide, silver chlorobromide, silver chloroiodide, silver iodobromide, and silver chloroiodobromide, but not limited thereto.

The silver halide grains may have a uniform halogen composition or a multiple structure varying in composition from the surface to the interior (see Japanese Patent Application Kokai Nos. 57-154232, 58-108533, 59-48755, and 59-52237; U.S. Pat. No. 4,433,048; and European Patent No. 100,984). When a silver halide is used alone without combining an organic silver salt-oxidizing agent, the silver chloroiodide, iodobromide, and

chloroiodobromide in which the X-ray pattern of silver iodide crystals is observable may preferably be used. For example, silver iodobromide of such nature is prepared by first adding silver nitrate solution to potassium bromide solution to form silver bromide particles and then adding potassium iodide to the mixture. Also useful are plate particles having a thickness of up to 0.5  $\mu\text{m}$ , a diameter of at least 0.6  $\mu\text{m}$ , and an average aspect ratio of at least 5 (see U.S. Pat. Nos. 4,414,310 and 4,435,499 and German Patent Application (OLS) No. 3,241,646A1) and monodispersed emulsion having approximately uniform grain size distribution (see Japanese Patent Application Kokai Nos. 57-178235, 58-100846, and 58-14829, International Publication No. 83/02332A1, European Pat. Nos. 64,412A3 and 83,377A1). Silver halide grains of epitaxial junction type may also be used (see Japanese Patent Application Kokai No. 56-16124 and U.S. Pat. No. 4,094,684). More than one silver halide having different crystal habit, halogen composition, grain size, or grain size distribution may also be used in admixture. More than one monodispersed emulsion having different grain size may be mixed so as to regulate gradation.

The silver halide used in the present invention preferably has an average grain size of from 0.001  $\mu\text{m}$  to 10  $\mu\text{m}$  and more preferably from 0.001  $\mu\text{m}$  to 5  $\mu\text{m}$ .

For the purpose of improving high or low intensity reciprocity law failure, there may be employed water-soluble iridium salts such as iridium (III, IV) chlorides and ammonium hexachloroiridate, and water-soluble rhodium salts such as rhodium chloride.

The silver halide emulsions may be applied without post-ripening, but ordinarily after chemical sensitization. For chemical sensitization purpose, there may be used sulfur sensitization, reducing sensitization, noble metal sensitization and other processes which are well known in connection with the emulsions for photosensitive materials of the ordinary type, and combinations thereof. Such chemical sensitization may be carried out in the presence of a nitrogen-containing heterocyclic compound as disclosed in Japanese Patent Application Kokai Nos. 58-126526 and 58-215644.

The silver halide emulsions used in the practice of the present invention may be either of the surface latent image type wherein latent images are predominantly formed on the grain surface or of the internal latent image type wherein latent images are formed in the grain interior. Also employable is a direct reversal emulsion having an internal latent image type emulsion combined with a nucleating agent.

The amount of the photosensitive silver halide coated preferably ranges from 1 mg/m<sup>2</sup> to 10 g/m<sup>2</sup> of silver.

In the practice of the present invention, an organic metal salt which is relatively stable to light may be used as an oxidizing agent in combination with the photosensitive silver halide. It is necessary that the photosensitive silver halide and the organic metal salt be in contact with or close to each other. Preferred among these organic metal salts are organic silver salts. The organic metal salt incorporated in a heat-developable photosensitive material in combination with the silver halide is believed to participate in redox reaction by the catalysis of a latent image of silver halide when the heat-developable photosensitive material is heated to a temperature of at least 80° C., preferably at least 100° C.

Exemplary of the organic compounds which can be used to form the above-mentioned organic silver salt oxidizing agents, there may be given aliphatic and aro-

matic carboxylic acids, thiocarbonyl-containing compounds having a mercapto group or alpha-hydrogen, imino-containing compounds, and the like.

Useful examples of the organic silver salt oxidizing agent are those described in Japanese Patent Application Kokai No. 58-58543, page 19, left-lower column to page 20, right-upper column.

In the present invention, there may be contained a compound which, when the photosensitive silver halide is reduced into silver at elevated temperatures, produces or releases a mobile or diffusible dye in direct or inverse proportion to the reaction. These compounds are simply referred to as dye-providing substances hereinafter.

Typical of the dye-providing substances which can be used in the present invention are couplers capable of reacting with a developing agent. Coupler based systems are such that oxidation-reduction reaction of a silver salt with a developing agent gives an oxidized form of developing agent which in turn, reacts with a coupler to form a dye, and many such systems are described in the literature. Illustrative examples of the developing agents and couplers are described in detail in, for example, T. H. James, "The Theory of the Photographic Process", 4th Ed., pages 291-334 and 354-361, and S. Kikuchi, "Photographic Chemistry", 4th Ed., Kyoritsu Publishing K.K., pages 284-295. Another class of dye-providing substances includes dye-silver compounds in which an organic silver salt is combined with a dye. Examples of the dye-silver compounds are described in Research Disclosure, May 1978, pages 54-58 (RD-16966).

A further class of dye-providing substance includes azo dyes which are generally used in the heat development silver dye bleaching process. Examples of the azo dyes and the bleaching process are described in U.S. Pat. No. 4,235,957 and Research Disclosure, April 1976, pages 30-32 (RD-14433) inter alia. Leuco dyes as described in U.S. Pat. Nos. 3,985,565 and 4,022,617 are further examples of the dye-providing substances.

A still further example of the dye-providing substances is a compound having the function of releasing or diffusing a diffusible dye imagewise.

The compounds of this type may be represented by the following formula [L I]:

(Dye-X)<sub>n</sub>-Y

[L I]

wherein Dye represents a dye group or a dye precursor group; X represents a simple bond or a connecting group; and Y represents a group which, in correspondence or counter-correspondence to photosensitive silver salt having a latent image distributed imagewise, produces a difference in diffusibility of the compound represented by (Dye-X)<sub>n</sub>-Y or releases Dye, the diffusibility of Dye released being different from that of the compound represented by (Dye-X)<sub>n</sub>-Y, and n represents an integer of 1 or 2, when n=2, the Dye-X's may be the same or different.

Exemplary of the dye-providing substances having general formula [L I] there may be given dye developing reagents in the form of a hydroquinone-type developing reagent having a dye moiety attached thereto as disclosed in U.S. Pat. Nos. 3,134,764; 3,362,819; 3,597,200; 3,544,545 and 3,482,972. In addition, substances which

release a diffusible dye through intramolecular nucleophilic substitution reaction are disclosed in Japanese Patent Application Kokai No. 51-63618 and substances

which releases a diffusible dye through intramolecular rewind reaction of an isooxazolone ring are disclosed in Japanese Patent Application Kokai No. 49-111628. In the systems to which these substances are applied, a diffusible dye is released or diffused where no development has taken place and no dye is released or diffused where development has taken place. 5

Since development and release or diffusion of the dye concurrently occur in these systems, it is very difficult 10 to obtain an image having a high S/N ratio. In order to overcome this drawback, another system is proposed wherein the dye-providing substance is previously modified into an oxidant form having no dye releasing ability so that the modified substance may coexist with a 15 reducing agent or precursor thereof. After development, the reducing agent which remains non-oxidized acts on the modified substance to reduce it, thereby releasing the diffusible dye. Typical examples of the 20 dye-providing substances usable in such a system are described in Japanese Patent Application Kokai Nos. 53-110827, 54-130927, 56-164342, and 53-35533.

Also known are substances which release a diffusible 25 dye where development has occurred. The substances which release a diffusible dye through the reaction of an oxidation product of a developing reagent with a coupler having a diffusible dye as an eliminatable group are described in British Pat. No. 1,330,524; Japanese Patent 30 Publication No. 48-39165; U.S. Pat. No. 3,443,940 and the like, and the substances which produce a diffusible dye through the reaction of an oxidation product of a developing reagent with a coupler having an anti-diffusible group as an eliminatable group are described in U.S. 35 Pat. No. 3,227,550 and the like.

The systems using these color developing agents have the serious problem that the resulting image can be 40 contaminated with oxidation decomposition products of a developing agent. To overcome this problem, a dye-releasing compound has been proposed which itself has a reducing ability without the need for a developing reagent. Typical examples of these compounds are presented below together with the patent or literature 45 disclosing them. The definition of legends in the formulas is given in the corresponding literature.



11

-continued



Any of the foregoing dye-providing substances may be used in the practice of the present invention.

Illustrative examples of the image-forming substances which may be used in the practice of the present invention are described in the foregoing patents which are incorporated herein by reference. Since mentioning all the preferred compounds is impossible and redundant, some are given below by way of illustration. For example, the dye-providing substances represented by general formula [L I] include the following compounds.

Exemplary of the dye-providing substances which can be used in the practice of the present invention there may be given those compounds described in the above-incorporated Japanese Patent Application Kokai No. 59-84236, pages 60-91, with the compounds identi-

12

fied therein as compound Nos. (1)-(3), (10)-(13), (16)-(19), (28)-(30), (33), (35), (38)-(40), and (42)-(64) being favorable among others. Also useful are the cyan and yellow dye-providing substances illustrated below.

5

Cyan-dye-providing substance



10

15



20

25

Yellow dye-providing substance



30

35

40

45

50

The above-illustrated compounds are only some examples of the useful dye-providing substances and not intended for limitation purpose.

In the practice of the present invention, the dye-providing substance may be introduced into a layer of photo-sensitive material by any well-known methods, for example, the method described in U.S. Pat. No. 2,322,027.

In this case, an organic solvent having a high boiling point or an organic solvent having a low boiling point as described below may be used.

For example, the dye-providing substance is first dissolved in a high-boiling organic solvent, for example, a phthalic acid alkyl ester (such as dibutyl phthalate, diethyl phthalate, etc.), a phosphoric acid ester (such as diphenyl phosphate, triphenyl phosphate, tricresyl phosphate, diethylbutyl phosphate, etc.), a citric acid

ester (such as tributyl acetyl citrate, etc.), a benzoic acid ester (such as octyl benzoate, etc.), an alkylamide (such as diethyl lauryl amide, etc.), a fatty acid ester (such as dibutoxyethyl succinate, dioctyl azelate, etc.), and a trimesic acid ester (such as tributyl trimesate, etc.); or an organic solvent having a low boiling point of about 30°C to 160°C, for example, a lower alkyl acetate (such as ethyl acetate, butyl acetate, etc.), ethyl propionate, sec-butyl alcohol, methyl isobutyl ketone, beta-ethoxyethyl acetate, methyl cellosolve acetate, cyclohexanone, etc. Mixtures of the above-described high boiling organic solvents and low boiling organic solvents may also be used. The solution of the dye-providing substance may then be dispersed in a hydrophilic colloid.

Further, it is possible to use a method for dispersion in 15 polymers as described in Japanese Patent Publication No. 51-39853 and Japanese Patent Application Kokai No. 51-59443. Moreover, various surface-active agents may be used when the dye-providing substance is dispersed in a hydrophilic colloid. For this purpose, the 20 surface-active agents illustrated in other part of the specification may be used.

The high-boiling organic solvent may be used in the 25 practice of the present invention in amounts of up to 10 grams, preferably up to 5 grams per gram of dye-providing substance.

In order to provide a wide range of color within the 30 chromaticity diagram using the three primary colors, yellow, magenta and cyan, the heat-developable photosensitive material used in the present invention should include at least three silver halide emulsion layers having 35 sensitivity in different spectra.

Typical combinations of at least three silver halide emulsion layers having sensitivity in different spectra are a combination of blue-sensitive emulsion layer/-green-sensitive emulsion layer/red-sensitive emulsion layer, a combination of green-sensitive emulsion layer/red-sensitive emulsion layer/infrared-sensitive emulsion layer, a combination of blue-sensitive emulsion layer/green-sensitive emulsion layer/infrared-sensitive emulsion layer, and a combination of blue-sensitive emulsion layer/red-sensitive emulsion layer/infrared-sensitive emulsion layer. By the infrared-sensitive emulsion layer used herein it is meant that the emulsion layer is sensitive to light having a wavelength of more 45 than 700 nm, particularly more than 740 nm.

The heat-developable photosensitive materials of the 50 present invention may have two or more emulsion layers having sensitivity in the same spectrum, but different in emulsion sensitivity.

Each of the above-mentioned emulsion layers and/or photo-insensitive hydrophilic colloid layer disposed adjacent thereto should contain either of a dye-providing substance which releases or forms a hydrophilic yellow dye, a dye-providing substance which releases or forms a hydrophilic magenta dye, and a dye-providing substance which releases or forms a hydrophilic cyan dye. Differently stated, each emulsion layer and/or a photoinsensitive hydrophilic colloid layer disposed adjacent thereto should contain a dye-providing substance which releases or forms a hydrophilic dye of different hue. If desired, mixtures of two or more dye-providing substances having the same hue may be used. When the dye-providing substance is originally colored, the heat-developable photosensitive material may preferably take such a layer arrangement as an arrangement of a blue-sensitive emulsion layer, a yellow dye-providing substance layer, a green-sensitive emulsion layer, a

magenta dye-providing substance layer, a red-sensitive emulsion layer, and a cyan dye-providing substance layer, and an arrangement of a green-sensitive emulsion layer containing a yellow dye-providing substance, a red-sensitive emulsion layer containing a magenta dye-providing substance, and an infrared-sensitive emulsion layer containing a cyan dye-providing substance, both from the exposure radiation incident side.

In order to impart color sensitivity as mentioned 10 above to the respective silver halide emulsions, each silver halide emulsion may be sensitized with a known sensitizing dye so as to provide the desired spectral sensitivity.

A reducing agent may desirably be used in the photosensitive material of the present invention. The reducing agents used herein include well-known reducing agents and the above-mentioned dye-providing substances having reducing ability. Also included are reducing agent precursors which themselves have no reducing nature, but exhibit reducing nature under the action of a nucleophilic agent or heat during the development process.

Examples of the reducing agents used herein include inorganic reducing agents such as sodium sulfite and sodium hydrogen sulfite, benzene sulfonic acids, hydroxylamines, hydrazines, hydrazides, boron-amine complexes, hydroquinones, aminophenols, catechols, p-phenylenediamines, 3-pyrazolidinones, hydroxytetroinic acids, ascorbic acids, 4-amino-5-pyrazolones, etc. and the reducing agents described in T.H. James, "The Theory of the Photographic Process", the Fourth Edition, pages 291-334. Also usable are reducing agent precursors as disclosed in Japanese Patent Application Kokai Nos. 56-138736 and 57-40245, U.S. Pat. No. 4,330,617, and the like. Various combinations of developing reagents as described in U.S. Patent No. 3,039,869 may also be used.

In the practice of the present invention, an image formation promotor may also be used. The image formation promoters have the functions of promoting such reaction as redox reaction of a silver salt-oxidizing agent with a reducing agent, formation of a dye from a dye-providing substance, decomposition of a dye or release of a mobile dye, and promoting transfer of a dye from a photosensitive material layer to a dye-fixing layer. From their physical-chemistry, they may be classified into bases, base precursors, nucleophilic compounds, oils, thermal solvents, surface-active agents, and compounds capable of interacting with silver or silver ion. It should be noted that these compounds generally have multiple functions and thus possess some of the above-mentioned promoting effects combined.

The image formation promoters are illustrated for each of functional classes. However, this classification is made for convenience of description and actually, one compound often possesses more than one function in combination.

(a) Bases

Preferred examples of the bases include (1) inorganic bases, for example, hydroxides, secondary and tertiary phosphates, borates, carbonates, quinolines, and metabolites of alkali metals and alkaline earth metals; ammonium hydroxides; quarternary alkyl ammonium hydroxides; and other metal hydroxides; and (2) organic bases, for example, aliphatic amines such as trialkyl amines, hydroxylamines, and aliphatic polyamines; aromatic amines such as N-alkyl-substituted aromatic amines, N-hydroxylalkyl-substituted aromatic amines

and bis[p-(dialkylamino)phenyl]methanes; heterocyclic amines, amidines; cyclic amidines; guanidines; and cyclic guanidines. The particularly preferred bases are those having a pKa value of 8 or higher.

(b) Base precursors

Base precursors are preferably those precursors which undergo any reaction under heat to release a base, for example, organic acid-base salts which are decomposed or decarbonated upon heating, and compounds which are decomposed to release amines through such reactions as intramolecular nucleophilic substituting reaction, Lossen rearrangement, Beckman rearrangement, etc. The preferred base precursors include salts of trichloroacetic acid as described in British Pat. No. 998,949; salts of alphasulfonylacetic acid as described in U.S. Pat. No. 4,060,420; salts of propionic acid as described in Japanese Patent Application No. 58-55700; 2-carboxylcarboxamide derivatives as described in U.S. Pat. No. 4,088,496; salts of thermally decomposable acids with a basic component containing an organic base and an alkali metal or alkaline earth metal as described in Japanese Patent Application No. 58-69597; hydroxamcarbamates utilizing Lossen rearrangement as described in Japanese Patent Application No. 58-43860; and aldoximcarbamates capable of forming nitriles upon heating as described in Japanese Patent Application No. 58-31614. In addition, base precursors as disclosed in British Pat. Nos. 998,945 and 2,079,480; U.S. Pat. No. 3,220,846; and Japanese patent application Kokai No. 50-22625, etc. are also useful.

(c) Nucleophilic compounds

Exemplary of the nucleophilic compounds there may be given water, water-releasing compounds, amines, amidines, guanidines, hydroxylamines, hydrazines, hydrazides, oximes, hydroxamic acid derivatives, sulfonamides, active methylene compounds, alcohols, and thiols, as well as salts and precursors of these compounds.

(d) Oils

Useful are those high-boiling organic solvents which are used as a solvent in emulsion dispersing a hydrophobic compound and also known as plasticizers.

(e) Thermal solvents

The thermal solvents are those compounds which are solid at an ambient temperature, but melts at approximately developing temperatures to serve as solvents. Useful are ureas, urethanes, amides, pyridines, sulfonamides, sulfones, sulfoxides, esters, ketones and ethers, provided that they are solid at temperatures of lower than 40° C.

(f) Surface-active agents

Typical surface-active agents are pyridinium salts, ammonium salts, and phosphonium salts as disclosed in Japanese Patent Application Kokai No. 59-74547, and polyalkylene oxides as disclosed in Japanese Patent Application Kokai No. 59-57231.

(g) Compounds capable of interacting with silver or silver ion

Useful are imides, nitrogen-containing heterocyclic compounds as disclosed in Japanese Patent Application No. 58-51657, thiols as disclosed in Japanese Patent Application No. 57-222247, thioureas, and thioethers.

These image formation promoters may be incorporated in the photosensitive material and/or the dye-fixing material. The particular layer into which the image formation promoters are incorporated may be any of the emulsion layer, intermediate layer, protective layer, image-receiving or dye-fixing layer, and layers adjoin-

ing any of these layers. The same applies to an embodiment where both the photosensitive layer and the dye-fixing layer are on a common support.

The image formation promoters may be used alone or in admixture of two or more. Generally, the promoting effect is enhanced by the use of more than one promoter. An outstanding promoting effect is obtained particularly when the base or base precursor is combined with another promoter.

In the practice of the present invention, a variety of development inhibitors may be used for the purpose of obtaining a consistent image irrespective of variations in treating temperature and time during heat development. By the development inhibitor is meant those compounds capable of, immediately after development has proceeded to an optimum extent, neutralizing or reacting with a base to reduce its concentration in the film to inhibit development, or those compounds capable of, immediately after optimum development, interacting with silver or silver salt to retard development. Illustrative examples are acid precursors capable of releasing acid upon heating, electrophilic compounds capable of substitution reaction with a coexisting base upon heating, nitrogen-containing heterocyclic compounds, mercapto compounds, and the like. Specific examples of the acid precursors are oxime esters as disclosed in Japanese Patent Application Nos. 58-216928 and 59-48305, and those compounds capable of releasing an acid through Lossen rearrangement as disclosed in Japanese Patent Application No. 59-85834. Specific examples of the electrophilic compounds capable of substitution reaction with a base upon heating are such compounds as disclosed in Japanese Patent Application No. 59-85836, etc. The effect of these development inhibitors is enhanced particularly when they are combined with base precursors. The proportion of the base precursor to the acid precursor used herein may preferably range from 1/20 to 20/1, and more preferably, from 1/5 to 5/1 in molar ratio.

Further, in the present invention, it is possible to use a compound which activates development simultaneously with stabilizing the image. Particularly preferred compounds used herein are isothiuroniums including 2-hydroxyethylisothiuronium trichloroacetate as described in U.S. Pat. No. 3,301,678; bisisothiuroniums including 1,8-(3,6-dioxaoctane)-bis(isothiuronium trichloroacetate) as described in U.S. Pat. No. 3,669,670; thiol compounds as described in German patent application (OLS) No. 2,162,714; thiazolium compounds such as 2-amino-2-thiazolium trichloroacetate, 2-amino-5-bromoethyl-2-thiazolium trichloroacetate, etc., as described in U.S. Pat. No. 4,012,260; and compounds having alpha-sulfonylacetate as an acid part such as bis(2-amino-2-thiazolium)-methylenebis(sulfonylacetate), 2-amino-2-thiazolium phenylsulfonylacetate, etc. as described in U.S. Pat. No. 4,060,420.

Also preferred are azothio ethers and blocked azothione compounds as described in Belgian Pat. No. 768,071; 4-aryl-1-carbamyl-2-tetrazoline-5-thione compounds as described in U.S. Pat. No. 3,893,859; and those compounds described in U.S. Pat. Nos. 3,839,041; phthalazinone, 2-acetylphthalazinone, 5-amino-1,3,4-thiadiazole-2-thiol, 3-mercaptop-1,2,4-triazole, bis(dimethylcarbamyl)disulfide, 6-methylthiouracil, 1-phenyl-2-tetrazoline-5-thione, and the like. Particularly effective toning agents are compounds which can impart a black color tone to images.

The content of such a toning agent as described above generally ranges from about 0.001 to 0.1 mole per mole of silver in the photosensitive material although the exact content depends upon the type of a heat developable photosensitive material used, processing conditions, desired images and various other factors.

In the practice of the present invention, the binders may be employed alone or in combinations thereof. The preferred binder used is a hydrophilic binder. The typical hydrophilic binder is a transparent or translucent hydrophilic binder, examples of which include natural substances, for example, proteins such as gelatin, gelatin derivatives and cellulose derivatives and polysaccharides such as starch, gum arabic etc.; and synthetic polymers, for example, water-soluble polyvinyl compounds such as polyvinyl pyrrolidone, acrylamide polymer, etc. Another example of the synthetic polymer compound is a dispersed vinyl compound in a latex form which is used for the purpose of increasing the dimensional stability of a photographic material.

The high-boiling organic solvent may be dispersed in the binder together with hydrophobic compounds, for example, a dye-providing substance such that the volume of the solvent is less than about 1 cc, preferably less than about 0.5 cc, and most preferably less than about 0.3 cc per gram of the binder.

In the heat-developable photosensitive material and the dye-fixing material according to the present invention, the photographic emulsion layer, conductive layers, dye-fixing layer and other binder layers may contain inorganic or organic hardeners. It is possible to use chromium salts such as chromium alum, chromium acetate, etc.; aldehydes such as formaldehyde, glyoxal, glutaraldehyde, etc.; N-methylol compounds such as dimethylolurea, methylol dimethylhydantoin, etc.; di-oxane derivatives such as 2,3-dihydroxydioxane, etc.; active vinyl compounds such as 1,3,5-triacryloyl-hexahydro-s-triazine, 1,3-vinylsulfonyl-2-propanol, 1,2-bis(vinylsulfonylacetamide)ethane, etc.; active halogen compounds such as 2,4-dichloro-6-hydroxy-s-triazine, etc.; mucohalogenic acids such as mucochloric acid, mucophenoxychloric acid, etc. or the like alone or in combinations of two or more.

The support used in the light-sensitive material of the present invention and the optional dye-fixing material must withstand the processing temperature. Exemplary of ordinary supports there may be given not only glass, paper, metal and analogues, but also an acetyl cellulose film, a cellulose ester film, a polyvinyl acetal film, a polystyrene film, a polycarbonate film, a polyethylene terephthalate film, and a film or plastic material related thereto. Further, a paper support laminated with a polymer such as polyethylene, etc. may be used. Those polyesters described in U.S. Pat. Nos. 3,634,089 and 3,725,070 are preferably used.

When a dye-providing substance which releases a mobile dye imagewise is used in the practice of the present invention, a dye transfer assistant may be used to transfer the dye from the photosensitive layer to the dye-fixing layer. The dye transfer assistants of the type supplied from outside the system include water and aqueous alkaline solutions containing sodium hydroxide, potassium hydroxide, or other inorganic alkali metal salts. Further, there may be used low boiling solvents such as methanol, N,N-dimethylformamide, acetone, diisobutyl ketone, etc., and mixtures of such a low boiling solvent with water or aqueous alkaline solution. The dye transfer assistant may be used by

wetting the image receiving layer with the transfer assistant.

When the dye transfer assistant has been incorporated into the heat-developable photosensitive material or dye-fixing material, the transfer assistant need not be supplied from the outside. The above-described dye transfer assistant may be incorporated into the material in the form of water of crystallization or microcapsules or as a precursor which releases a solvent at elevated temperatures. More preferably, a hydrophilic thermal solvent which is solid at an ambient temperature and melts at a high temperature may be incorporated into heat-developable photosensitive material or dye-fixing material. The hydrophilic thermal solvent may be incorporated in the heat-developable photosensitive material and/or the dye-fixing material. Although the solvent can be incorporated into any of the emulsion layer, intermediate layer, protective layer, and dye-fixing layer, it is preferred to incorporate it into the dye-fixing layer and/or layers adjacent thereto.

Examples of the hydrophilic thermal solvents include ureas, pyridines, amides, sulfonamides, imides, alcohols, oximes and other heterocyclic compounds.

When the dye-providing substance having general formula (L I) as defined above is contained in the heat-developable photosensitive material of the present invention, such additives as anti-irradiation and antihalation substances and various dyes need not necessarily be contained in the photosensitive material because of coloring of the dye-providing substance. For the purpose of improving the sharpness of an image, filter dyes, absorptive materials and the like may be contained as disclosed in Japanese Patent Publication No. 48-3692; U.S. Pat. Nos. 3,253,921; 2,527,583; and 2,956,879; etc. Preferred among these dyes are thermally decoloring dyes, for example, those disclosed in U.S. Pat. Nos. 3,769,019; 3,745,009; and 3,615,432.

The heat-developable photosensitive materials of the present invention may optionally contain any of a variety of additives well known for use in heat-developable photosensitive materials and possess in addition to the photosensitive layer, any layers including protective layer intermediate layer, AH layer, and release layer. Examples of the additives include such additives as disclosed in Research Disclosure, Vol. 170, June 1978, No. 17029, for example, plasticizers, sharpness improving dyes, AH dyes, sensitizing dyes, matte agents, surface-active agents, brightening agents, discoloration retarders, etc.

When the photographic elements according to the present invention contain a dye-providing substance which forms or releases a dye upon heat development. They are generally classified into two typical forms, one form having photosensitive and dye-fixing layers 55 separately applied on two separate supports and another form having both photosensitive and dye-fixing layers applied on a common support.

The former system having photosensitive and dye-fixing layers separately applied on two separate supports is generally sub-classified into two types, peeling type and non-peel type. In the case of peeling type, the coated surface of the photosensitive element is overlapped the coated surface of the dye-fixing element after imagewise exposure or heat development, and the photosensitive element is separated from the dye-fixing element immediately after formation of a transfer image. Depending on whether the final image is of reflective or transmissive type, the support of the dye-fixing

element may be selected among opaque or transparent supports. If desired, a white reflective layer may be applied. In the case of non-peel type, a white reflective layer must be interposed between the photosensitive layer of the photosensitive element and the dye-fixing layer of the dye-fixing element while the white reflective layer may be applied to either the photosensitive element or the dye-fixing element. The support of the dye-fixing element must be transparent support.

The latter system having both light-sensitive and dye-fixing elements applied on a common support is typically one wherein the photosensitive element need not be peeled from the image-receiving element after formation of a transfer image. In this case, a photosensitive layer, a dye-fixing layer, and a white reflective layer are laminated on a transparent or opaque support. The preferred arrangements are transparent or opaque support/photosensitive layer/white reflective layer/-dye-fixing layer and transparent support/dye-fixing layer/white reflective layer/photosensitive layer, to 20 name a few.

Another typical form having both light-sensitive and dye-fixing elements applied on a common support is one wherein a release layer is applied at a proper location such that the photosensitive element may be entirely or partially separated from the dye-fixing element, as disclosed in Japanese Patent Application Kokai No. 56-67840, Canadian Pat. No. 674,082, and U.S. Pat. No. 3,730,718.

When the non-peel type is employed, the conductive layer according to the present invention is disposed at such a position as not to obstruct exposure and image observation.

The dye-fixing element optionally used in the present invention has at least one layer containing a mordant. When the image-receiving or dye-fixing layer is positioned at the surface, a protective layer may further be applied thereon if necessary.

Further, in order that a dye transfer assistant may be contained in a sufficient amount or controlled, a water-absorbing layer or dye transfer assistant-containing layer may be provided. Such a layer may be applied contiguous to the dye-fixing layer or via an intermediate layer.

The dye-fixing layer used in the practice of the invention may be divided into two layers containing mordants having different mordanting power, if necessary.

The mordants contained in the dye-fixing layer is not particularly limited although polymeric mordants are particularly preferred. The polymeric mordants include polymers containing a tertiary amino group, polymers having a nitrogen-containing heterocyclic moiety, and polymers containing a quaternary cationic group.

Those polymers containing vinyl monomer units having a tertiary amino group are described in Japanese Patent Application Nos. 58-169012 and 58-166135. Those polymers containing vinyl monomer units having a tertiary imidazole group are described in Japanese Patent Application Nos. 58-226497 and 58-232071; U.S. Pat. Nos. 4,282,305; 4,115,124; and 3,148,061. Those polymers containing vinyl monomer units having a quaternary imidazolium salt are described in U.K. Pat. Nos. 2,056,101; 2,093,041; and 1,594,961; U.S. Pat. Nos. 4,124,386; 4,115,124; 4,273,853; and 4,450,224; and Japanese patent application Kokai No. 48-28225. Those polymers containing vinyl monomer units having a quaternary ammonium salt are described in U.S. Pat. Nos. 3,709,690; 3,898,088; and 3,958,995; Japanese pa-

tent application Nos. 58-166135, 58-169012; 58-232070, 58-232072, and 59-91620.

The dye-fixing element used in the practice of the present invention may include any auxiliary layer, for example, a release layer, matte agent layer, and anti-curling layer.

One or more of the above-mentioned layers may contain a base or base precursor for promoting dye transfer, hydrophilic thermal solvent, anti-discoloration agent for preventing discoloration of dyes, UV absorber, dispersed vinyl compound for increasing dimensional stability, and brightening agent.

The binders used in the above-mentioned layers are preferably hydrophilic, and typically transparent or translucent hydrophilic colloids. Exemplary of the hydrophilic binders there may be given natural substances, for example, proteins such as gelatin, gelatin derivatives, cellulose derivatives, etc., and polysaccharides such as starch, dextrin, pluran, gum arabic, etc., and synthetic polymers, for example, water-soluble polyvinyl compounds such as polyvinyl alcohol and polyvinyl pyrrolidone, acrylamide polymers, etc. Particularly useful among them are gelatin and polyvinyl alcohol.

The dye-fixing element may further include in addition to the above-mentioned layers, a reflective layer containing a white pigment like titanium oxide, neutralizing layer, neutralization timing layer or the like depending on the intended application. These layers may also be provided in the heat-developable photosensitive element as well as in the dye-fixing element. The organization of these reflective, neutralizing, and neutralization timing layers is described, among others, in U.S. Pat. Nos. 2,983,606; 3,362,819; 3,362,821; and 3,415,644; and Canadian Pat. No. 928,559.

The light source for image exposure to record an image in the heat-developable photosensitive material may be any radiation including visible light. In general, light sources used in ordinary color printing may be used, for example, tungsten lamps, mercury lamps, halogen lamps like iodine lamps, xenon lamps, laser sources, CRT sources, fluorescent lamps, light emitting diodes (LED), and the like.

The temperature at which the heat-developable photosensitive materials are heated during heat development process ranges from about 80° C. to about 250° C., preferably from about 110° C. to about 180° C., more preferably above about 140° C., and most preferably above about 150° C. in the preferred range. To carry our transfer of a dye image, the heating temperature during the transfer process ranges from room temperature to the temperature used in the heat development process, and preferably up to a temperature 10° C. lower than the heat development temperature. Heating means additionally used during the development or transfer process may be any suitable heating means other than the conductive layer according to the present invention, for example, a simple heat block, an iron, a heat roller and the like.

When water is used as the dye transfer assistant, a water softener is used in order to prevent calcium and magnesium ions in water from forming a precipitate to cause nonuniform dye transfer. Preferred examples of the water softeners which may be added for this purpose include organic phosphonic acid compounds; polyphosphoric acid compounds as exemplified by sodium hexametaphosphate, sodium tetrapolyphosphate, sodium tripolyphosphate or potassium salts of these polyphosphoric acids; aminopolycarboxylic acids as

exemplified by ethylenediamine tetraacetic acid, nitro-tri-acetic acid, triethylenetetramine hexa-acetic acid, iminodiacetic acid, hydroxyethyliminoacetic acid, N-hydroxymethyl-ethylenediamine triacetic acid, diethylenetriamine pentaacetic acid, cyclohexanediamine tetraacetic acid, and diaminopropanol tetraacetic acid. The amount of water softener added is not particularly limited and usually determined in accordance with the hardness of water. Generally, the water softener is added in an amount of 0.001 to 30 grams, preferably 0.01 to 10 grams per liter of water. No particular limit is imposed on the temperature of water although warm water can accelerate transfer rate.

#### BENEFITS OF THE INVENTION

Since at least two exothermic conductive layers are provided on a support according to the present invention, there is obtained a photographic element for use in a heat-developable photographic material having conductive and photographic layers can prevent adhesion between adjoining conductive and photographic layers or between adjoining conductive layers during shelf storage with such photographic material pieces placed one on another.

The additional or auxiliary conductive layer protects the surface of the exothermic conductive layer having the function of a heating element to prevent marring and crazing due to physical contact, pressure or other factors.

When the additional or auxiliary conductive layer protecting the primary conductive layer is resistant to humidity, the dependency of electric resistance on humidity is also improved.

These features allow for stable and uniform heat development and heat transfer of a mobile dye.

#### EXAMPLES

Examples of the present invention are presented below by way of illustration and not by way of limitation.

##### EXAMPLE 1

A coating dispersion of carbon black was prepared by roughly dispersing carbon black having a DBP oil absorption of 350 cc/100 grams with the aid of a dispersant in the following formulation and then treating in a colloid mill for further dispersion.

| Ingredient                                                                | Amount    |
|---------------------------------------------------------------------------|-----------|
| Carbon black (particle size 15 m $\mu$ , DBP oil absorption 350 cc/100 g) | 45 grams  |
| Demor N <sup>1</sup>                                                      | 5 grams   |
| Nissan nonion NS208.5 <sup>2</sup> , 5% in water                          | 54 ml     |
| Water                                                                     | 700 ml    |
| 10% gelatin solution                                                      | 600 grams |
| 10% 2-ethylhexyl succinate                                                | 90 cc     |
| sodium sulfonate in 1/1 water/methanol                                    |           |

<sup>1</sup>manufactured by Kao Atlas K.K.

<sup>2</sup>manufactured by Nissan Chemical K.K.

The dispersion was applied onto a polyethylene terephthalate film to a wet thickness of 80  $\mu$ m and dried to form a conductive layer, obtaining sample A.

The above-prepared dispersion was combined with each of the following addition solutions and then applied onto sample A to a wet thickness of 40  $\mu$ m and

dried to form an auxiliary layer, obtaining samples B to E.

| Sample | Addition solution composition                                                                                                                  |
|--------|------------------------------------------------------------------------------------------------------------------------------------------------|
| B      | 5% solution of polyvinyl alcohol having polymerization degree of 2000<br>10% gelatin solution<br>Water                                         |
| C      | 5% solution of polyvinyl alcohol having polymerization degree of 1500<br>5% solution of polyvinyl pyrrolidone<br>10% gelatin solution<br>Water |
| D      | 10% gelatin solution<br>SiO <sub>2</sub> powder (particle size 3-5 $\mu$ m)<br>Water                                                           |
| E      | 10% gelatin solution<br>Graphite powder (particle size 3-5 $\mu$ m)<br>Demor N (Kao Atlas K.K.)                                                |

Then, a photosensitive layer and a protective layer (this combination is referred to as a photographic layer, hereinafter) were applied onto samples A to E on the opposite side to the conductive layer with respect to the support of polyethylene terephthalate film, obtaining photosensitive materials.

The photosensitive silver halide emulsion, silver benzotriazole emulsion, and dye-providing substance dispersion used in the preparation of the photographic layer were prepared by the following procedures.

##### [Photosensitive Silver Halide Emulsion]

An aqueous gelatin solution was prepared by dissolving 40 grams of gelatin and 26 grams of KBr in 3,000 ml of water. The solution was agitated while keeping at 50° C.

Then 34 grams of silver nitrate in 200 ml of water was added to the solution over a period of 10 minutes. The resulting silver iodobromide emulsion was adjusted to such pH as to remove an excess salt by precipitation. The emulsion was then adjusted to pH 6.0, obtaining a silver iodobromide emulsion in a yield of 400 grams.

##### [Silver Benzotriazole Emulsion]

In 3000 ml of water were dissolved 28 grams of gelatin and 13.2 grams of benzotriazole. The solution was agitated at 40° C.

A solution of 17 grams of silver nitrate in 100 ml of water was added to the solution over a period of 2 minutes. The resulting silver benzotriazole emulsion was adjusted to such pH that an excess salt precipitated, and the excess salt was filtered off. The emulsion was then adjusted to pH 6.3, obtaining a silver benzotriazole emulsion in a yield of 400 grams.

##### [Dye-Providing Substance Dispersion]

Five (5) grams of dye-providing substance (A) having the formula shown below was added to a mixture of 10 grams of tricresyl phosphate and 30 ml of ethyl acetate and heated at about 60° C. into a solution. The solution was mixed by agitation with 100 grams of 10% gelatin solution and 10 ml of 5% aqueous solution of sodium p-alkylbenzene sulfonate (C<sub>12-13</sub>alkyl), and the mixture was dispersed with a homogenizer for 10 minutes at 10,000 rpm. This dispersion is designated dye-providing substance dispersion.

Dye-providing substance (A), chemical formula:



The procedure of applying the photographic layer is described below.

A photosensitive layer having the following formulation was applied to the rear surface of the support of each sample A to E prepared as above.

#### Photosensitive Coating Composition

| Photosensitive coating composition                     |                                        |  |
|--------------------------------------------------------|----------------------------------------|--|
| (a) Silver iodobromide emulsion                        | 20 grams                               |  |
| (b) Silver benzotriazole emulsion                      | 10 grams                               |  |
| (c) Water                                              | 3.5 ml                                 |  |
| (d) Dye-providing substance (A) dispersion             | 33 grams                               |  |
| (e) 5% aqueous solution of compound having the formula | 5 ml                                   |  |
|                                                        | <chem>C9H19-C6H4-O-(CH2CH2O)8-H</chem> |  |
| (f) 10% guanidine trichloroacetate in ethanol          | 12.5 ml                                |  |
| (g) 10% dimethylsulfamide in water                     | 4 ml                                   |  |

Components (a) to (g) were mixed into a coating solution, which was applied to the rear surface of the polyethylene terephthalate film to a wet thickness of 30  $\mu\text{m}$  and then dried to form a photosensitive layer. The following composition was further applied thereon as a protective layer.

#### Protective Composition

|                                                         |          |  |
|---------------------------------------------------------|----------|--|
| (h) 10% gelatin in water                                | 35 grams |  |
| (i) 10% guanidine trichloroacetate in ethanol           | 5 ml     |  |
| (j) 1% 2-ethylhexyl succinate sodium sulfonate in water | 4 ml     |  |
| (k) Water                                               | 56 ml    |  |

Components (h) to (k) were mixed into a coating solution, which was applied to a wet thickness of 25  $\mu\text{m}$  and then dried, obtaining a photosensitive material.

The thus obtained photosensitive materials which correspond to samples A, B, C, D, and E are designated photosensitive materials I, II, III, IV, and V, respectively.

Each of these photosensitive materials I to V was cut into sheet-like pieces which were placed one on another. A shelf test was effected by keeping the stack

under a load of 100 g/cm<sup>2</sup> for one day in a room at a temperature of 25° C. and a relative humidity of 75%.

In photosensitive material I using sample A, the conductive and photographic layers were fused together so that they could not be separated. In photosensitive materials II to V using samples B to E, the conductive and photographic layers were readily separated, demonstrating that the present invention is effective in preventing adhesion.

#### EXAMPLE 2

Samples F to I were prepared by applying the following coating solutions on sample A to a wet thickness of 40  $\mu$  and drying to form an auxiliary layer.

| Sample | Solution (or dispersion) composition              |           |
|--------|---------------------------------------------------|-----------|
| F      | 10% polyvinyl butyral in isopropanol              | 100 grams |
|        | Acetylene black (particle size 20 $\mu\text{m}$ ) | 2 grams   |
| G      | 10% cellulose diacetate in acetone                | 100 grams |
|        | Furnace black (particle size 20 $\mu\text{m}$ )   | 2 grams   |
| H      | 10% cellulose triacetate in methylene chloride    | 100 grams |
|        | Furnace black (particle size 80 $\mu\text{m}$ )   | 3 grams   |
| I      | 5% polycarbonate in methylene chloride            | 200 grams |
|        | Furnace black (particle size 20 $\mu\text{m}$ )   | 2 grams   |

The procedures of Example 1 were repeated by applying a photosensitive layer onto the support surface opposite to the conductive layer and subjecting a stack of cut pieces to a shelf test. It was observed that the photosensitive materials from samples F to I were effective in preventing adhesion or keeping separate their photographic and conductive layers.

#### EXAMPLE 3

Samples A, B, and F to I prepared in Examples 1 and 2 were measured for electric resistance under varying humidity to determine the variation of electric resistance with humidity. The electric resistance was first measured in a room at a temperature of 25° C. and a relative humidity (RH) of 40%. The samples were then allowed to stand for 30 minutes in a room at a temperature of 25° C. and a relative humidity of 80%, and the electric resistance was again measured at 25° C. and RH 80%. The ratio of resistance at RH 80% to resistance at RH 40% is shown below.

| Sample | Resistance ratio (80%/40% RH) |
|--------|-------------------------------|
| A      | 2.40                          |
| B      | 1.95                          |
| F      | 1.25                          |
| G      | 1.30                          |
| H      | 1.10                          |
| I      | 1.05                          |

As seen from this data, the auxiliary layers containing a hydrophobic polymer as the binder (samples F to I) are effective in improving the humidity dependency of electric resistance.

#### EXAMPLE 4

Samples J and K were prepared by applying the following coating solutions on sample A from Example 1 to a wet thickness of 40  $\mu\text{m}$  and drying to form an auxiliary layer.

| Sample | Solution composition                            |           |
|--------|-------------------------------------------------|-----------|
| J      | 10% gelatin in water                            | 250 grams |
|        | Tricresyl phosphate                             | 25 grams  |
|        | 5% sodium dedecylbenzene sulfonate in water     | 100 ml    |
|        | Furnace black (particle size 40 $\mu\text{m}$ ) | 5 grams   |
|        | $\text{H}_2\text{O}$                            | 600 ml    |
| K      | 10% gelatin in water                            | 450 grams |
|        | Dibutyl phthalate                               | 10 grams  |
|        | 5% sodium dedecylbenzene sulfonate in water     | 100 ml    |
|        | Furnace black (particle size 40 $\mu\text{m}$ ) | 5 grams   |
|        | $\text{H}_2\text{O}$                            | 400 ml    |

Samples A, J and K were subjected to a bending test wherein the sample was bent at varying angles. Crazing occurred less frequently in samples J and K than in sample A. It was demonstrated that the conductive layer including at least two layers according to the present invention is effective in preventing crazing.

These results clearly show the significant improvements by the present invention.

I claim:

1. A photographic element comprising at least two exothermic electroconductive layers and at least one layer selected from a photosensitive layer and an image-receiving layer on a support, where upon heat developing the photosensitive layer, or transferring a mobile dye resulting from heat-development of the photosensitive layer to an image-receiving layer, or conducting such heat-development and dye transfer at the same time, electricity is applied to at least one of the electroconductive layers to generate heat, wherein at least one layer of said at least two exothermic electroconductive layers is an exothermic electroconductive layer having the function of a heating element on which at least an auxiliary exothermic electroconductive layer is formed.

2. A photographic element according to claim 1 wherein said exothermic electroconductive layer hav-

ing the function of a heating element has an electric resistance corresponding to a volume resistance of  $10^{-4}$  to 10 ohm-cm.

3. A photographic element according to claim 1 wherein the auxiliary exothermic electroconductive layer has an electric resistance corresponding to a volume resistance of  $10^{-1}$  to  $10^4$  ohm-cm.

4. A photographic element according to claim 1 which further comprises at least a silver halide, a binder, and a dye-providing substance on the support.

5. A photographic element according to claim 1 which is a dye-fixing material having a dye-fixing layer on the support.

6. A photographic element according to claim 1, wherein an electrode is attached to at least said exothermic electroconductive layer having the function of a heating element.

7. A photographic element according to claim 1, wherein said exothermic electroconductive layers comprise conductivity imparting fine particles dispersed in a binder.

8. A photographic element according to claim 7, wherein said conductivity imparting fine particles are selected from the group consisting of metals, metal alloys, silicon carbide, molybdenum silicide, oxide semiconductors, graphite and carbon black.

9. A photographic element according to claim 7, wherein said conductivity imparting fine particles are selected from the group consisting of graphite and carbon black.

10. A photographic element according to claim 7, wherein said binder is hydrophilic.

11. A photographic element according to claim 10, wherein said binder is gelatin.

12. A photographic element according to claim 10, wherein said conductivity imparting fine particles are used in an amount of from 10 to 90% by weight in the binder.

13. A photographic element according to claim 9, wherein said graphite or carbon black is used in an amount of from 15 to 85% by weight in the binder.

14. A photographic element according to claim 1, wherein said at least one auxiliary exothermic electroconductive layer has an electrical resistance at least  $1\frac{1}{2}$  fold higher than that of the exothermic electroconductive layer having the function of a heating element.

15. A photographic element according to claim 1, wherein the at least one layer is said photosensitive layer.

16. A photographic element according to claim 1, wherein the at least one layer is said image-receiving layer.

17. A photographic element according to claim 1, wherein said at least one auxiliary exothermic electroconductive layer is provided on the exothermic electroconductive layer having the function of a heating element in direct contact therewith.

\* \* \* \* \*